

Patented Nov. 6, 1923.

1,473,510

# UNITED STATES PATENT OFFICE.

CHARLES E. PARSONS, OF ENGLEWOOD, NEW JERSEY.

## PROCESS OF PRODUCING CARBIDES OF SODIUM AND BORON.

No Drawing.

Application filed April 10, 1923. Serial No. 681,214.

To all whom it may concern:

Be it known that I, CHARLES E. PARSONS, a citizen of the United States, residing at Englewood, in the county of Bergen and State of New Jersey, have invented certain new and useful Improvements in Processes of Producing Carbides of Sodium and Boron; and I do hereby declare the following to be a full, clear, and exact description of the invention, such as will enable others skilled in the art to which it appertains to make and use the same.

This invention relates to a process of simultaneously producing sodium and boron carbides from sodium tetraborate,  $Na_2B_4O_7$ , and carbon, and has for its object to provide a procedure which will be more efficient in action and less costly to carry out than those heretofore proposed.

With these and other objects in view, the invention consists in the novel steps and combinations of steps constituting the process, all as will be more fully hereinafter disclosed and particularly pointed out in the claims.

In carrying out this invention, one may take any suitable quantity of sodium tetraborate,  $Na_2B_4O_7$ , heat the same to about 880° C., or until it is melted, and then raise the molten mass to a temperature above 1000° C., or better still to about 1200° C., or to a point just safely under its dissociation temperature. To the superheated melt thus had, one now adds an excess of finely divided carbon, such as anthracite coal, coke or charcoal, which is thoroughly admixed with the melted borate and the temperature raised until substantially all the sodium present sublimes off in the form of a carbide leaving boron carbide behind in accordance with the following equation:



The lower boron carbide  $B_6C$  is not directly made by this process so long as a state of fusion exists unless the temperature exceeds 1700° C. It is preferred to make the higher carbide  $B_4C_3$  by the above disclosed fusion process and to then convert it into the hard dissociation product  $B_6C$  by a separate procedure.

Of course, the operation of producing simultaneously sodium and boron carbides in the manner above stated must be carried out in a closed system; otherwise the so-

dium carbide  $Na_2C_2$  will in contact with the air be burned to sodium carbonate. It is also essential that the sublimed sodium carbide be condensed and cooled out of contact with the air.

The boron carbide  $B_4C_3$  can be tapped out of the furnace in the usual manner. It is important that the carbon be not added to the molten borate until the latter has been heated several hundred degrees above its melting point for otherwise elemental sodium is liable to be driven off and the lower carbide  $B_6C$  instead of the higher carbide  $B_4C_3$  is liable to be produced.

That is, the higher boron carbide  $B_4C_3$  does not dissociate while in the molten bath under the hydrostatic pressure of the fusion, and the latter also prevents elemental sodium from leaving the borate and escaping as a sublimate before uniting with the carbon.

It is of course possible to dissociate the boron carbide  $B_4C_3$  without removal from the furnace chamber by raising the temperature of said carbide to say about 1700° C. after the sodium carbide has been removed by sublimation. By this means, the boron carbide  $B_4C_3$  may be broken back to the lower carbide  $B_6C$ .

What is claimed is:

1. The process of making a boron carbide which consists in melting sodium tetraborate,  $Na_2B_4O_7$ ; raising the temperature of the molten bath to a point above 1000° C.; adding sufficient carbon to said bath to produce the desired boron carbide; and recovering the product.

2. The process of simultaneously producing sodium carbide and boron carbide from sodium tetraborate, which consists in melting said borate out of contact with the air; raising the temperature to a point between 1000° C. and the point of dissociation of said borate; adding sufficient carbon to produce the desired sodium and boron carbides; and recovering said carbides.

3. The process of simultaneously making sodium carbide  $Na_2C_2$  and boron carbide  $B_4C_3$  which consists in melting in a closed system sodium tetraborate  $Na_2B_4O_7$ ; raising the temperature of the molten bath thus produced to a point below that at which said borate will decompose; adding sufficient carbon to the bath to produce the desired sodium carbide and boron carbide; and

segregating and recovering said carbide products out of contact with the air.

4. The process of producing a boron carbide which consists in melting sodium tetraborate; raising the temperature of the melt to a point below that of its dissociation temperature; adding sufficient carbon to pro-

duce a higher carbide of boron; still further raising the temperature until said higher carbide dissociates into a lower carbide; and 10 recovering the latter.

In testimony whereof I affix my signature.

CHARLES E. PARSONS.